

C. L. REIZENSTEIN.  
METHOD OF DECORATING GLASSWARE.  
APPLICATION FILED JULY 16, 1917.

1,251,577.

Patented Jan. 1, 1918.

2 SHEETS—SHEET 1.

FIG. 1



FIG. 2



FIG. 3



FIG. 4



FIG. 5



INVENTOR

Charles L. Reizenstein  
By Kay Zetter Paole  
Attorney

C. L. REIZENSTEIN.  
METHOD OF DECORATING GLASSWARE.  
APPLICATION FILED JULY 16, 1917.

1,251,577.

Patented Jan. 1, 1918.  
2 SHEETS—SHEET 2.

FIG. 6



FIG. 7



FIG. 8



INVENTOR

Charles L. Reizenstein  
By Kay Lotten Powell  
Attorneys

# UNITED STATES PATENT OFFICE.

CHARLES L. REIZENSTEIN, OF PITTSBURGH, PENNSYLVANIA.

## METHOD OF DECORATING GLASSWARE.

1,251,577.

Specification of Letters Patent.

Patented Jan. 1, 1918.

Application filed July 16, 1917. Serial No. 180,786.

*To all whom it may concern:*

Be it known that I, CHARLES L. REIZENSTEIN, a citizen of the United States, and resident of Pittsburgh, in the county of Allegheny and State of Pennsylvania, have invented a new and useful Improvement in Methods of Decorating Glassware; and I do hereby declare the following to be a full, clear, and exact description thereof.

10 My invention relates to an improved method of ornamenting glassware. In general the invention comprises forming an ornamental background applied to the rear or underside or inside of the glass vessel covering a certain field, and opposite this background or field on the outer face of the vessel applying an ornamental design comprising portions of colored glass which cover portions of the field, while the remainder of 20 the field shows through to the background, whereas the other portions of the field are partially or entirely covered by ornamentation on the face.

In the embodiment of my invention here selected for illustration, and referring to the drawings, Figure 1 is a fragmentary section of a glass dish which is to be treated in accordance with the method embodying the invention; Fig. 2 is a fragmentary view 30 showing the design partly completed; Fig. 3 is a like view showing a further development of the design; Fig. 4 is a further view showing a still further development; Fig. 5 is a like view of the complete design; Figs. 35 6 and 7 are views of other embodiments of the invention; and Fig. 8 is a detached ornamented portion made according to the invention.

In carrying out the invention, the face 40 1 of the border or rim of the glass vessel is colored or etched in any desired manner to produce a scroll or other design 2. The etching of the face however, is omitted in the areas 3 around the border. The under- 45 side of the rim, as at 4, is then treated with suitable coloring matter to form a solid background throughout the portion of the glass vessel which is to be ornamented. This colored background has two functions. 50 First, it forms a background or field for the colored glass areas 3 and the glass in these areas gives this background coloring a glazed or glossy appearance. Furthermore, the solid colored background forms a basis 55 or backing for enriching the coloring matter, which is applied to the raised orna-

mented part or border. For example, the area 5 of the border may be gilded or treated with some other suitable coloring matter over the etched pattern. To this colored 60 face of the border the background coloring matter will give an enriched finish. After applying the coloring matter to the rear face of the border to form the background in the areas 3, and after applying the coloring 65 matter to the areas 5 over the etched pattern, the coloring matter of these areas may be baked to set them permanently on the dish, or if it is desired to place some sort of ornamentation on the faces of the areas 70 3 this may be done in the following manner, for example: If it is desired to apply a design of flowers and foliage on the faces of these areas 3, such design may be formed in relief by applying suitable enamel in the 75 areas 6 shown in white Fig. 4. This preliminary foundation for the ornamentation for the areas 3 may be subjected to the baking process at the same time that the colored background and colored faces of the border 80 are baked.

The areas 6 so treated may be then colored in imitation of flowers and foliage, etc., and the vessel again subjected to a suitable baking process to set this variegated coloring of the flowers and foliage.

While I have shown my method of ornamenting glassware applied simply to a border of a glass vessel, it is to be understood that the same method may be employed in ornamenting any other portion of the vessel, such for example, as the center of a dish, or entire border and center. For example in Fig. 6 I have shown a plate with a simple border illustration applied on the 95 rear or bottom side 10 and defining outlines 11 applied on the outer side. In Fig. 7 I have illustrated a jug having the coloring field 12 on the rear or inner side and the ornamentation 13 applied on the outer face. 100 In Fig. 8 I have shown a detached ornamentation having the colored portion 14 applied on the rear face and the ornamentation 15 applied so as to leave exposed through the glass a portion of the rear coloring 105 14.

It is to be understood, however, that the invention contemplates a method of ornamenting the glass which will present an ornamental colored background for certain or 110 all areas of the glass, and as a further development and in combination with such

background, the face of the glass vessel is also ornamented and finally the ornamentation upon the face of the glass vessel may be varied by inclusion of colored glass areas 5 or fields showing through to the colored background.

While I have shown here a particular example of my invention, it is to be understood that the same may be altered in details and 10 in arrangement of the designs within the scope of the appended claims.

What I claim is:

1. The method of ornamenting glassware which consists in applying to the rear or 15 under face of the glassware a suitable coloring matter covering a desired field thereof, applying colored ornamentation to the face of said glassware opposite said background and baking the same to give said background 20 and ornamentation a permanent set.

2. The method of ornamenting glassware which consists in applying to the rear or 25 under face of the glassware a suitable coloring matter covering a desired field thereof, applying colored ornamentation to the outer face of the glassware while omitting the ornamentation in certain parts opposite the ornamental background, and baking the same to give said background and ornamentation 30 a permanent set.

3. The method of ornamenting glassware which consists in applying to the rear or 35 under face of the glassware a suitable coloring matter covering a desired field thereof, ornamenting the outer face above said colored glass field partially by applying a foundation material to certain areas which are to be ornamented, then baking the vessel to set the background and ornamented face there-

of, applying suitable coloring to the foundation material in said colored glass areas, and again baking the vessel to set such coloring matter.

4. The method of ornamenting glassware, 45 which consists in applying to the rear or under-face of the glassware a suitable coloring matter covering a desired field thereof, preparing the outer face by applying a foundation material to certain areas which are to be ornamented, then baking the vessel to set 50 the background and said prepared outer face, applying suitable coloring matter to the outer face including said prepared areas, and again baking the vessel to set 55 such coloring matter.

5. The method of ornamenting glassware, which consists in applying to the rear or under-face of the glassware a suitable coloring matter covering a desired field thereof, 60 applying suitable colored ornamentation to the outer face of the vessel, baking the vessel to set the background and ornamented face thereof.

6. The method of ornamenting glassware, 65 which consists in applying to the rear or under-face of the glassware a suitable coloring matter covering a desired field thereof, applying suitable colored ornamentation to the outer face of the vessel including the 70 area opposite the background, and then baking the vessel to set the background and ornamented face thereof.

In testimony whereof I, the said CHARLES L. REIZENSTEIN, have hereunto set my hand.  
CHARLES L. REIZENSTEIN.

Witnesses:

JOHN F. WILL,  
J. R. KELLER.

Copies of this patent may be obtained for five cents each, by addressing the "Commissioner of Patents.  
Washington D. C."